

L. B. TEBBETTS, 2D.  
PROCESS FOR MAKING METAL INGOTS.  
APPLICATION FILED DEC. 4, 1917.  
1,298,825.

Patented Apr. 1, 1919.

Fig. 1.



Fig. 2.



Attest.  
Charles A. Becker.

Invention  
Lewis B. Tebbetts, 2D.  
By Ripley & Kingsland  
His Attorneys.

# UNITED STATES PATENT OFFICE.

LEWIS B. TEBBETTS, 2D, OF ST. LOUIS, MISSOURI.

## PROCESS FOR MAKING METAL INGOTS.

1,298,825.

Specification of Letters Patent.

Patented Apr. 1, 1919.

Application filed December 4, 1917. Serial No. 205,360.

To all whom it may concern:

Be it known that I, LEWIS B. TEBBETTS, 2d, a citizen of the United States, residing at the city of St. Louis and State of Missouri, have invented a new and useful Process for Making Metal Ingots, of which the following is a specification.

This invention relates to a new and useful process for making metal ingots adapted for 10 rolling into sheets.

Heretofore it has been the practice that metals such as aluminum, antimonial lead, lead, brass, copper, tin alloys and the like were cast into rolling ingots in upright 15 molds open at the top. When such ingots are cast a shrinkage hole is formed in the top edge of the ingot surrounding which shrinkage hole there is formed an area of defective metal containing impurities and 20 being of a porous or spongy character. When such ingots are rolled into sheets there has been a substantial wastage of metal by reason of the necessity of discarding that portion of the sheet in which the area surrounding the shrinkage hole in the ingot is 25 formed.

It is known in casting ingots that a shrinkage hole occurs where the metal cools last. It has therefore been impractical heretofore 30 to cast ingots in flat molds for the reason that a shrinkage hole would occur in the center of the top face of the ingot so that when such an ingot was rolled into sheets the defective portion of the sheet would be 35 in the center thereof.

An object of the invention is to provide a method of casting ingots in flat molds and cooling the mass of the metal within the mold from the center outwardly, so that the 40 outside of the ingot will be the last to cool thereby eliminating a shrinkage hole formation in the ingot, producing an ingot of uniform formation throughout so that there will be no wastage of metal when such ingots 45 are rolled into sheets.

The accomplishment of this object, as well as other advantages, is effected by the process hereinafter disclosed. The process consists in casting the metal in a flat open 50 mold and cooling the ingot from the center

outwardly by applying a cooling agent at the center of the molten mass so that the outer edges of the ingot will be the last to cool.

In the drawing I have illustrated an apparatus which is effective for satisfactorily producing the process of the invention, it being understood, however, that the principle of the process may be carried into effect by other apparatus.

In the drawing Figure 1 is a plan view of the apparatus; and,

Fig. 2 is a side elevation thereof.

In the drawing an open flat mold 1 is arranged above a water conduit 2 provided 65 with an upright nozzle 3 arranged to eject a volume of water against the bottom of the mold upon an area at the center thereof. For convenience, the conduit 2 may be controlled by a valve 4.

The metal is poured into the mold which is of thin sheet metal and will remain in a molten state for a sufficient period of time to permit the impurities in the metal to rise to the top and to be skimmed off, after 75 which the cooling agent is applied, cooling the mass from the center outwardly. The resulting ingot will be free from impurities and no shrinkage hole will be formed therein.

What I claim and desire to secure by Letters Patent, is:—

1. The process of casting ingots having smooth surfaces and suitable for rolling into sheets consisting in pouring the molten metal 85 into open flat molds and cooling the same by applying a cooling agent at a point substantially at the center of the bottom of the mass.

2. The process of casting metal ingots 90 having smooth surfaces and suitable for rolling into sheets which consists in pouring the molten metal into an open top flat mold, allowing the impurities to rise to the top of the mold, and then applying a cooling agent 95 to the center of the bottom of the mass whereby the same is cooled from the center outwardly.

LEWIS B. TEBBETTS, 2d.